

## UNITED STATES PATENT OFFICE

2,313,529

## FOG INHIBITOR FOR PHOTOGRAPHIC EMULSIONS

George E. Fallesen and John A. Leermakers,  
Rochester, N. Y., assignors to Eastman Kodak  
Company, Rochester, N. Y., a corporation of  
New Jersey

No Drawing. Application August 9, 1941,  
Serial No. 406,172

5 Claims. (Cl. 95—7)

This invention relates to fog inhibitors for photographic emulsions and to photographic emulsions containing them.

It is known that photographic emulsions particularly ultra-sensitive emulsions, or those containing color sensitizers exhibit a tendency to form a deposit of silver in the emulsion. This deposit extends more or less uniformly over the entire emulsion and is known as fog. Photographic fog is of two types, local and general. Local fog is formed by exposure of the film or plate at undesired points, as by a light leak in the camera. General fog or, as it is sometimes known, chemical fog, is formed in a number of ways. It may be caused by the conditions under which the film or plate is stored, such as conditions of high temperature or unusually long time of storage. The nature of the emulsion may also produce chemical fog, as well as the conditions of development of the emulsion, as by development for protracted periods of time or at temperatures above normal. Highly sensitive emulsions are more likely to fog than those of lower sensitivity. We are concerned primarily with general or chemical fog.

The primary object of the present invention is to provide anti-fogging or fog inhibiting agents for ultra-sensitive photographic emulsions and to thereby increase the stability of the emulsions. A further object is to provide anti-fogging agents which do not markedly lower the sensitivity of the emulsion.

These objects are accomplished by incorporating in the emulsion an acetylamino phenol or diacetylamino phenol.

These compounds are incorporated in a fast negative emulsion particularly a silver halide emulsion which contains optical sensitizing dyes. The emulsion used may be one which is intended to be used directly after emulsification or one which is subjected to ripening.

The following examples illustrate compounds which we have found suitable for inhibiting fog in photographic emulsions.



30 We have found that in the case of the monoacetylaminophenols the anti-foggant action is least in the ortho compounds, greater in the para compounds and greatest in the meta compounds. This is also true in general of the diacetylamino phenols. The effect of the compounds on photographic speed was also found to be related to the position of the substituents and to the number of acetyl groups in the compounds. The desensitizing effect was observed to be greater with the monoacetylamino phenols than with the diacetylamino phenols. The amount of desensitization caused by the diacetylamino phenols was found to be practically negligible and under most conditions these compounds seem to be very useful antifogants.

35 The antifoggant action was determined by incubation of the emulsions under simulated tropical conditions for two weeks and also by incubation for a similar length of time in dry heat at 50, 120° F. The results of the latter tests are tabu-

lated here for comparison with the initial fog in the emulsions with and without the antifoggants.

and X-ray emulsions. If used with sensitizing dyes they may be added to the emulsion before or

| Name of compound                              | Initial fog            |                           | 14-day 120° F. incubation fog |                           |
|-----------------------------------------------|------------------------|---------------------------|-------------------------------|---------------------------|
|                                               | Emulsion with compound | Emulsion without compound | Emulsion with compound        | Emulsion without compound |
| Acetyl m-amino-phenol, 8.3 grams per liter    | { Unsens<br>Pan. sens. | .03<br>.04                | .04<br>.07                    | .25<br>.16                |
| Acetyl p-amino-phenol, 8.33 grams per liter   | { Unsens<br>Pan. sens. | .04<br>.04                | .04<br>.07                    | .26<br>.19                |
| Diacetyl-o-amino-phenol, 4.16 grams per liter | { Unsens<br>Pan. sens. | .03<br>.07                | .04<br>.09                    |                           |
| Diacetyl m-amino-phenol, 4.16 grams per liter | { Unsens<br>Pan. sens. | .04<br>.05                | .04<br>.08                    | .12<br>.14                |
| Diacetyl p-amino-phenol, 4.16 grams per liter | { Unsens<br>Pan. sens. | .04<br>.06                | .03<br>.07                    | .12<br>.17                |
|                                               |                        |                           |                               | .45<br>.65                |

In the above table "Unsens." means an unsensitized emulsion and "Pan. sens." means a panchromatically sensitized emulsion. The amount of fog was determined by reading the density at the toe of the curve after exposure and development of the emulsions, in the usual manner.

The amount of the fog inhibiting agents used in the emulsion will depend upon the composition of the agent and upon the type of emulsion. In general, the amount of fog inhibiting agent used will vary from 1 gram to 10 grams per 1000 cc. of wet emulsion. It will be understood that more or less than this amount may be used. Generally, however, if a greater amount is used in the emulsion either no increased fog inhibiting effect is obtained or there is a decrease in the sensitivity of the emulsion. These compounds may be incorporated by mixing them with any suitable solvent which is inert with respect to the emulsion such as water, methyl alcohol, ethyl alcohol, acetone, and others.

The fog inhibiting agents which we have described may be used in various kinds of photographic emulsions. In addition to being useful in ordinary non-sensitized emulsions, they may be used also in orthochromatic, panchromatic

after the dyes are added. Various silver salts may be used as the sensitive salt such as silver bromide, silver iodide, silver chloride, and mixtures of these. The dispersing agent may be gelatin or other colloid such as collodion, albumen, cellulose organic derivatives or synthetic resins.

It is to be understood that we contemplate as included within our invention all modifications and equivalents falling within the scope of the appended claims.

We claim:

1. A gelatino-silver halide emulsion containing as an antifoggant a diacetylaminophenol.
2. A gelatino-silver halide emulsion containing a diacetylaminophenol in fog inhibiting amounts.
3. A gelatino-silver halide emulsion containing as an antifoggant diacetyl-m-aminophenol.
4. A gelatino-silver halide emulsion containing as an anti-foggant diacetyl-p-aminophenol.
5. A gelatino-silver bromide emulsion containing as an antifogulant approximately 4 grams per liter of diacetyl-m-amino phenol.

GEORGE E. FALLESEN.  
JOHN A. LEERMAKERS.